# EUROPEAN PATENT SPECIFICATION

(11) **EP 1 709 383 B1**
(45) Date of publication and mention of the grant of the patent: **18.04.2007**
(21) Application number: 05701286.6
(22) Date of filing: 28.01.2005
(51) Int. Cl.: F28F 9/18, B21D 39/06

(54) **METHOD FOR FORMING A WELDED CONNECTION BETWEEN A TUBESHEET AND A NUMBER OF TUBES AND A DEVICE PRODUCED BY SUCH METHOD**
VERFAHREN ZUR HERSTELLUNG EINER GESCHWEISSTEN VERBINDUNG ZWISCHEN EINEM ROHRBODEN UND MEHREREN ROHREN SOWIE DURCH SOLCH EIN VERFAHREN HERGESTELLTE VORRICHTUNG
PROCEDE DE REALISATION D'UNE LIAISON SOUDEE ENTRE UNE PLATINE A TUBES ET LES TUBES, ET DISPOSITIF AINSI OBTENU

(30) Priority: 28.01.2004 EP 04075261
(43) Date of publication of application: 11.10.2006
(73) Proprietor: Madioen Holding B.V., 4033 AV Lienden (NL)
(72) Inventor: VAN DEN BOOM, Jacobus, Elfridus, NL-4003 DZ Tiel (NL)
(74) Representative: Grootscholten, Johannes A.M.
(86) International application number: PCT/EP2005/000952
(87) International publication number: WO 2005/075923

(56) References cited:
- US-A- 2 405 399
- US-A- 3 207 215
- US-A- 3 628 923
- US-A- 3 841 938
- PATENT ABSTRACTS OF JAPAN vol. 011, no. 054 (M-563), 19 February 1987 (1987-02-19) -& JP 61 216821 A (HITACHI LTD), 26 September 1986 (1986-09-26)

## Description

The present invention according to a first aspect relates to a method for performing a welded connection between a tubesheet and at least one tube.

According to a second aspect the present invention relates to a device produced by the method according to the invention. Such a device finds application in e.g. heat exchangers. However, a useful application in other technical fields is not excluded.

In related heat exchangers there is an exchange in heat between the medium that runs through the tubes and the medium flowing at the outer side of the tubes. To ensure that these two media are separated and remain to be so seperated from each other, adequate tube to tubesheet connections have to be executed, e.q. by expanding the tube ends.

In those cases in which the usage of the heat exchanger requires extra certainty that the tube-tubesheet connections will be leak tight, tubes are welded to the tubesheet, like in US-3,628,923.

An important characteristic of the welded connection is that the welds must provide a sufficiently long leak path. The person skilled in the art will be familiar with the term leak path, being the shortest way of the end of the crevice between tube and bore to the medium inside the tube seen through the weld.

The weld-connections provided by the prior art methods are characterised by the fact that the weld-connection is made by melting the edge of the tubesheet-borezone together with the relatively thin tube-ends, which operation is very critical in terms of amongst others a) fulfilment of specified minimum leak path at all weldpositions, b) avoiding damage or penetration of the tube end by e.g. a welding-arc, c) avoiding the blocking of a centering-device, used for automated welding, at removal due to a narrowing of the tube diameter caused by the weld, etcetera.

The invention is aimed at providing a method for forming a connection between a tubesheet and a tube, wherein the welding operation is far less critical. This object is reached by the method according to the invention which comprises:
- providing a tube sheet with a first surface and a second surface and a number of bores extending from the first surface to the second surface,
- providing the tube of a pliable or at least deformable material with an exterior shape and dimensions, which shape and dimensions enable the tube to be accommodated in a corresponding bore,
- placing the tube in the corresponding bore, such that an end portion of the tube protrudes from the side of the first surface of the tube sheet,
- forming an end portion of the tube into at least a flare,
- making a welded connection between the tube sheet and the tube at the circumference of the flare, after placing the tube.

The invention is distinguished particularly in that flaring the protruding end portion comprises: compressing the protruding end portion axially relative to the length direction of the tube and thus obtaining a compressed end portion of increased thickness.

In the method according to the invention the weld arc is aimed on the circumference of the flare and tubesheet itself, at a distance, e.g. several millimeters away from the edge of the tubesheet-bore zone. This makes the welding operation far less critical. Especially in cases where the wall of material of the tube is thin, and a welding operation could pierce the wall, the invention is beneficial, since providing the additional thickness can prevent such piercing of said wall.

In the method according to the invention the leak path is freely and better controllable opposed to the traditional welding details. This because the size of the welded connection is freely controllable as the weld arc is aimed at the circumference of the flare and the tubesheet itself at the end portion of increased thickness.

Due to the fact that the weld-arc is now aimed at the circumference of the flare of increased thickness and the tubesheet, damage or penetration or piercing of the tube-end is less likely to occur. Also the possibility of a centering device getting blocked in the tube is avoided, as the welded connection does not influence the tube diameter.

Furthermore, the new method according to the invention provides benefits for execution of re-tubing. Retubing is some times executed to replace leaking tubes of a heat exchanger. Such leakage may occur after prolonged operation of the heat exchanger, especially when operated under harsh conditions (e.g. very corrosive media).

In the re-tubing execution of the tubes connected to the tubesheet with the traditional weld details it is often necessary to clean up the bores due to local contamination that easily may influence the welding process in a negative way. Such clean up is normally executed by grinding the inner surface of the bores. Thus the diameter of the bores may run out of tolerance which influences the fit of the new tubing.

With the method according to the present invention retubing of a heat exchanger does not require cleaning of the bores in order to remove contaminations. It is sufficient to grind the first surface of the tubesheet to remove any contamination which might be present.

In the method according to the invention a tubesheet with a first surface and a second surface is provided. The tubesheet can be formed by any material which can be subjected to a welding operation and which has suitable properties for the intended use. A selection of a suitable material is within the knowledge of the skilled person. Examples of suitable materials can be selected from metals and metal alloys, such as (stainless) steel, nickel (alloys), copper (alloys), titanium (alloys), zirconium. The material of the tubesheet may be cladded or coated with a material which is more corrosion resistant then the base material, wherein cladding or coating may be executed prior or subsequent to assembly with the tube(s). Suitable cladding materials may be selected from the group consisting of stainless steel, nickel (alloys), copper (alloys), titanium (alloys).

The tubesheet is provided with a number of bores extending from the first surface to the second surface. These bores can be circular, in correspondence with the tubes, but these tubes may have any other desired shape or form in transverse section, e.g. rectangular, along with the bores. Within this specification and the claims it is to be understood that the wording "a number of" refers to at least one, viz. one or more, in all instances that it is used. The bores can be provided by any suitable technique known to the skilled person, such as drilling. Preferably the bore has a diameter, shape, form or other dimensions, which enables standard tubes to be placed in the bore. The selection of suitable diameters, shapes, forms or dimensions of the bore in connection with the tubing used is within the knowledge of the skilled person. Suitable guides are given in tables RCB-7.41 and RCB-7.41 M of the eight edition of the standards of the Tubular Exchanger Manufacturers Association.

The number of tubes provided in the method according to the invention have an exterior diameter, shape, form or other dimension, which enables the tube to be placed in a bore. This can be either with a tight fit, a loose fit, or a temperature dependent fit. A temperature dependant fit can be reached by cooling the pipe prior to fitting it into the bore, or heating the tubesheet prior to fitting the tube into the bore. Preferably the tube is of a type which is commercially readily available. It is to be understood that the invention is not limited to the use of a specific type of tube.

The provided tubes are made from a pliable material, which enables them to be flared and compressed axially at their ends. Any pliable material can be used, as long as it can be subjected to a welding operation as well as deformation or other operation to provide a flare. The selection of suitable materials is within the knowledge of the skilled person. Examples of suitable materials can be selected from the group comprising metals, metal alloys, such as (stainless) steel, nickel (alloys), copper (alloys), titanium (alloys), zirconium.

Flaring of the end of the protruded portion of the tube can be done by any suitable methods known to the skilled person, e.g. by using a compressing tool. Preferably the flares are made by hydraulic pressing or forming.

It must be understood that if the other end of a tube is freely movable through the bore, flaring can be done before a tube is placed in the bore. If the other end of a tube does not permit passage through the bore, flaring will be done after the tube is placed in a bore.

The welded connection between the tubesheet and each tube, is made at the circumference of each flare. The welded connection can be made by using known welding techniques and equipment. It is possible to make the welded connection in a single passage of the weld arc around the circumference of the flare. During such a single welding passage the material of the tube and the tubesheet is melted together. During such a single welding passage preferably welding material is deposited to strengthen the welded connection. In addition to this in the method according to the present invention deposition of weld material will increase the leak path. However, such deposition of weld material is not strictly obligatory since for some applications the melting operation will provide a welded connection with sufficient strength and leak path.

It is also possible to use multiple welding passages, such as two or three or more welding passages. Such additional welding passages can be used to further strengthen the welded connection. When multiple welding passages are used, all welding passages can be similar or different welding modes can be used. For instance, when two welding passages are used, the first welding passage can be used to prepare the path for the second welding passage by e.g. evening it to provide a smooth surface. In such a case the first welding passage only melts the material of the tubesheet and the tube together, and none or little filler material is deposited. During the second subsequent welding passage, welding material is deposited.

After the second welding passage it is possible to use a third welding passage in order to melt the deposited welding material in order to improve the weld shape. The use of such a third weld passage may provide a welded connection with a flattened surface. If electric welding is used preferably the third welding passage is then performed with a higher voltage than the previous welding passages.

In an embodiment of the invention, the method comprises: providing a recess in the tube sheet at the circumference of the bore at the first surface, the recess in shape and dimensioning essentially corresponding with the compressed end portion of the tube. As an advantage the flare, i.e. compressed end portion of the tube, can be placed in the recess to obtain an essentially even first surface, with which the outer rim of the compressed end portion of the tube is in line. The operation to be described below of smoothing the first surface can thus be simplified considerably.

According to a preferred embodiment of the method according to the invention, the flares are provided with a trumpet shape or a cone shape. It is also possible that the form of the flare is a combination of a cone shape and a trumpet shape. In such a case the trumpet shape is located closer to the circumference of the flare, than the cone shape. The trumpet shape or cone shape or the combined trumpet-cone shape of the flare provides a smooth flow of a fluid medium when accessing or leaving the pipe.

According to a different preferred embodiment of the method according to the invention the end of the bore at the first surface is rounded and/or has the shape of a cone. Such a shape of the bore end facilitated flaring the tube in a trumpet shape, a cone shape or a combined trumpet-cone shape.

A preferred embodiment of the method according to the invention comprises: mechanically interconnecting the tube and the tube sheet at the latest prior to welding the flared protruding end portion of the tube, thus providing a preliminary positional fixation of the tube and the tube sheet relative to one another to be maintained during at least one of the operations of flaring the protruding end portion of the tube and welding the flare to the tube sheet. As a consequence the mutual positioning of the tubes and the tube sheet is ensured, even when during subsequent operations like flaring and welding the relative mutual positioning may be endangered without the said mechanical fixation. In such an embodiment, especially when the provided tube has a loose fit in the bore, it is preferred to expand the tube to fit tightly in at least a part of the bore. This operation is performed preferably prior to performing the flaring operation on the end of the tube or at least (at the latest) prior to welding. The expanded tight fit of the tube in at least a part of the bore fixates the tube in the bore which is beneficial for the flaring operation and/or the welding operation.

In a preferred embodiment of the method according to the invention a groove is provided in the corresponding bore, which groove extends from the first surface in the axial direction of the bore over at least a portion of the axial length thereof. In such an embodiment the tube has a tight fit in the bore, in the part where the groove is located, over a distance shorter then the axial length of the groove. The groove can be made in any form. A suitable form for making the groove is by making a screw thread. This because making a screw thread is a technique which is well known and for which many suitable devices are available. The inventive function of the groove is to provide an open channel for a fluid between the second surface and the first surface despite the tight fit of the pipe in at least a part of the bore over a distance shorter then the axial length of the groove. Further it is note here that an internal screw thread shaped groove in the bore can be employed in combination with an external screw thread on the outer surface of the tube to provide a mechanical interconnection between the tube sheet in the bore and the tube. The tube can then be screwed into the bore, and in such an embodiment the open channel can still be realised, provided the screwed interconnection is sufficiently loose to allow passage of expanding gasses and sufficiently fixed at the same time to allow for subsequent flaring and/or welding without the risk of misalignment of the tubes and the tube sheet during flaring and/or welding.

The presence of a groove in or on the internal surface of the bore prevents blowing up of the weld material during welding, especially when closing the weld around the flare, as there remains an open channel between the bore and the tube leading to the second surface, along which channel any gas near the area subjected to welding, that expands as a result of the heat generated by the welding operation, can escape. In an embodiment, wherein the tube is expanded, the groove can also perform the function of providing a suitable grip for the expanded tube, without closing the open channel Even if the groove does not extend through the bore, all the way to the second surface, the channel is not closed in an embodiment, wherein the tube is expanded only over a distance from the first surface, which distance is shorter than the length of the groove.

The groove or at least the open channel also makes it possible to conduct pressure using Non-Destructive Testing (NDT) to test if the welded connection of the tube to the sheet is sufficient leak tight. Examples of such pressure using NDT methods are the so called "soap test", a Helium leak test, and a pressure test. As these NDT methods are known to the skilled person they will be discussed below only briefly.

A suitable NDT method is the soap test in which a light air-over pressure is made around the tubes on the side of the second surface. The welds are than provided with a soap solution. On leaking, soap bubbles will develop which show the leak position.

Another suitable NDT is the He-leak test. In this test a light over-pressure of Helium gas is applied around the tubes on the side of the second surface. Subsequently the welded connections are sniffed with special equipment, which is able to detect break trough of the very penetrable helium.

A third suitable NDT is the pressure test. With this test water pressure is applied around the tubes on the side of the second surface. The level of the water pressure is related to the design pressure of the tube-tubesheet assembly. During the test the pressure is monitored and leakage is detected by any observed pressure drop event or any visual leakage.

After performing the pressure-using NDT method the remaining part of the tube not having a tight fit in the bore may be fitted tightly in the bore. This can be done by e.g. expanding the part of the tube not having a tight fit to fit tightly in the bore. During the expanding operation care is taken to avoid expanding of any part of the tube located outside the bore. In practice this can be achieved by not expanding the remaining 2-7 mm e.g. 5 mm of the tube located in the bore near the second surface. Hereby the channel formed by the groove is closed off. This provides additional sealing of the tube to tubesheet connection.

When more than one pipe and more than one bore are provided, it is beneficial if the bores are provided at such a distance of each other, that when the ends of the pipes are flared, the circumferences of the flares come in such proximity of each other that the welded connection at adjacent flares overlap. In this way a continuous surface is formed by the flares and the welded connections. Such a continuous surface forms a coverage over the tubesheet and can have the function of a cladding layer. Thus in applications in which the use of a cladded material for the tubesheet is suitable, the cladding layer may be formed by the continuous surface formed by the flares of the tubes and the welded connections. Any part of the tubesheet not covered by the continuous surface may be cladded in the usual way, or otherwise covered with a protective layer.

In order to form a smooth surface, the continuous surface formed by the flares and the welded connections is ground to a smooth surface and preferably subsequently polished. The presence of such a smooth continuous surface is beneficial in special applications wherein it is undesired if surface imperfections e.g. crevices etc. are present on the surface of the tubesheet. This e.g. provides a better septic quality of the tubesheet and in particular the tubesheet-bore-zone.

According to another aspect the present invention relates to a device produced in accordance with the method to which the present invention relates, comprising:
- a tubesheet with a first surface and a second surface and a number of circular bores extending from the first surface to the second surface,
- a number of tubes of a pliable material placed in each bore, wherein each tube has a flared portion on the side of the first surface, which flared portion with increased thickness is welded at its circumference to the first surface of the sheet.

The device according to the invention finds application in heat exchangers, although application in other technical fields is not excluded.

The tube sheet can be provided with a recess at the circumference of the bore at the first surface, the recess in shape and dimensioning essentially corresponding with the compressed end portion of the tube.

According to a preferred embodiment of the device according to the invention, the flares are provided with a trumpet shape or a cone shape. It is also possible that the form of the flare is a combination of a cone shape and a trumpet shape. In such a case the trumpet shape is located closer to the circumference of the flare, than the cone shape. The trumpet shape or cone shape or the combined trumpet-cone shape of the flare provides a smooth flow of a fluid medium when accessing or leaving the tube.

According to a different preferred embodiment of the device according to the invention the end of the bore at the first surface is rounded and/or has the shape of a cone. Such a shape of the bore end facilitates flaring the tube in a trumpet shape, a cone shape or a combined trumpet-cone shape.

It is preferred that the tube has a tight fit in at least a part of the bore. The tight fit of the tube in at least a part of the bore fixates the tube in the bore which is beneficial for the flaring operation and/or the welding operation. Furthermore, the tight fit provides additional sealing of the tube to tubesheet connection.

In a preferred embodiment of the device according to the invention a groove is located in the surface of the bore, which groove extends from the first surface in the axial direction of the bore for at least a portion of the axial length of the bore. In this case the tube can have a tight fit in the bore, in the part where the groove is located, over a distance shorter then the axial length of the groove. The function of the groove is to provide an open channel for a fluid between the second surface and the first surface despite the tight fit of the pipe in at least a part of the bore over a distance shorter then the axial length of the groove.

The presence of such a groove in the surface of the bore makes it possible to conduct pressure using Non-Destructive Testing (NDT) to test if the welded connection of the tube to the tubesheet is sufficient leak tight. Examples of such pressure using NDT methods have been discussed above.

It will be evident to the skilled person that the embodiment of the device according to the invention wherein there remains an open channel between the first surface and the second surface is not (optimally) suited for use in a heat exchanger. However, this embodiment is an important intermediate state in the production of a heat exchanger on which pressure using NDT methods can be performed. In order to make this embodiment of the device suitable for the application in a heat exchanger it is of importance to ensure that the tube has a tight fit over substantially the full axial length of the bore. If the tight fit of the tube in the bore is obtained by expanding the tube in the bore, in practice the remaining 2-7 mm e.g. 5 mm of the tube located in the bore near the second surface will remain unexpanded to prevent that any part of the tube located outside the bore is expanded.

The groove can have any form. A suitable form of the groove is a screw thread. This because making a screw thread is a technique which is well known and for which many suitable devices are available.

In a preferred embodiment of the device according to the invention more then one bore and more then one tube are provided and the welded connections between adjacent flares overlap. This embodiment of the device according to the invention comprises a continuous surface formed by the flares and the welded connections. Such a continuous surface forms a coverage over the tubesheet and can have the function of a cladding layer. Thus in application in which the use of a cladded material for the tubesheet is suitable, the cladding layer may be formed by the continuous surface formed by the flares of the tubes and the welded connections. Any part of the tubesheet not covered by the continuous surface may be cladded in the usual way, or otherwise covered with a protective layer.

Preferably the continuous surface is an even and smooth surface. Such an even and smooth surface is beneficial in special applications wherein it is undesired if surface imperfections such as crevices etc. are present on the surface of the tubesheet. This e.g. provides a better septic quality of the tubesheet, in particular the tubesheet-bore-zone.

The invention will be further explained with reference to the figures showing non-limiting embodiments of the invention, in which the same or similar parts and components are designated with the same reference numerals.

Figures 1A-1D show cross sectional overviews of welded tubesheet to tube connections according to the prior art.

Figures 2A-2C show cross sectional overviews of different stages of the method according to the invention.

Figure 3 shows a cross sectional overview along the line III-III in fig. 4 of a preferred embodiment of the device according the invention.

Figure 4 shows a plan overview of a preferred embodiment of the device according to the invention.

Figures 5A-5B, 6A-6B, 7A-7B show different embodiments of the inventions.

Figure 1A shows a cross sectional overview of a so called "seal weld" known from the art. This figure shows a tube 1 located in a bore of a tubesheet 2. The end 3 of the tube 1 is melted together with the tubesheet 2 by the weld arc 4. In this weld detail the weld 5 is formed by a single passage of the weld arc, whereby mostly just a little amount of weld-filler material is added or none at all. Although this weld detail is popular because of the relatively low costs for machining, it has the disadvantage that the weld penetration is relatively small, which makes that the leak path is in principle also relatively small.

Figure 1B shows an alternative "seal weld". In this alternative the tubesheet 2 is provided with a circular incision 6 around the bore. The incision 6 ensures a larger weld penetration. Moreover it effects that the tubesheet gets less change on distortion by weld-shrinkage-forces, due to the fact that these forces more easily can be reduced by relaxation. The appliance of a stringent set of weld parameters such as velocity, current, voltage stays very important to ensure that a sufficient leak path is obtained.

Figure 1C shows a so called "strength weld". The tube 1 is located in the bore of a tubesheet 2. The end of the bore is enlarged relative to the rest of the bore. The tube 1 is fitted into the bore up to the enlarged section of the bore. The tube end 3 is melted together with the tubesheet by the weld arc 4 under suppliance of weld-filler-material by supply means 7. Usually the welding is performed by two weld passages, of which formation of the root layer 8 is the most critical part of the welding process. The benefit of this weld detail opposed to those shown in figures 1A and 1B, is that the leak path can be better controlled.

Figure 1D shows a so called "fillet weld" which is only applicable for relatively thick tubes, to avoid that the weld arc punctures the wall of the tube. The tube 1 is located in the bore of the tubesheet 2, such that it protrudes with its end 3 above the first surface 10 of the tubesheet 2. Again the end of the bore of the tubesheet 2 is enlarged and the weld connections 8,9 are made in two welding passages in the enlarged part of the bore. Here too formation of the root layer 8 is the most critical part of the welding process.

Now, turning to a preferred embodiments of the present invention, figure 2A shows a tubesheet 2 with a first surface 10 and a second surface 11. The tubesheet 2 is provided with a bore 12, in which a screw thread 13 as an embodiment of a groove is formed. The screw thread 13 starts from the first surface 10 and extends in the axial direction of the bore 12 towards the second surface 11. The axial length of the screw thread is shorter than the axial length of the bore. A tube 1 with an external diameter, that enables it to be placed in the bore 12 with a loose fit, is provided and placed in the bore by moving it in the direction of the arrow. In an embodiment with an external screw thread on the outer surface of the tube, the tube can be screwed into the bore.

Figure 2B shows the position of the tube 1 in the bore 12 of the tubesheet 2, after it has been expanded to fit tightly in a portion of the bore, which portion is shorter than the axial length of the groove 13. As shown, the end 3 of the tube 1 protrudes above the first surface 10 of the tubesheet 2. The end of the bore in this situation is relatively unworked. However, it may be rounded of or have a trumpet, cone or a combined trumpet-cone shape. As the tube 1 remains to have a loose fitting in the bore on the side nearer to the second surface 11, there remains a connection 14 or open channel from the second surface 11 with the groove 13 and thus with the area subjected to welding. Thus there is a free channel for passage of a fluid, especially gasses expanding as a result of heat generated with the welding operation, between the second surface 11 and the first surface 10.

Figure 2C shows the next step in the method according to the invention. As is shown, the protruding end 3 of the tube 1 is flared and compressed to have an increased thickness, whereby a flare 20 is formed. At the circumference 21 of the flare, the welded connection is made with the weld arc 4 under suppliance of filler material by supply means 7.

Figure 3 shows a cross sectional overview along the lines III-III as shown in figure 4 of a preferred embodiment of the device according to the invention. As is shown the remaining unexpanded part of the tube is expanded to provide a tight fit of the tube 1 in the bore 12 over essentially the entire length thereof. Thereby the connection 14 is closed off. As is also shown, the bores 12 in the tubesheet 2 are provided at a distance such that the flares 20 come in such proximity of each other that adjacent welds 22 overlap. Thus, a continuous surface is formed by the flares 20 and the overlapping welds 22. This surface may be ground to an even surface and further polished to a smooth surface (not shown in figure 3).

Figure 4 shows a plan overview of a preferred embodiment of the device according to the invention. The device contains multiple tubes 1 connected to a tubesheet 2. At the first surface 10 of the tubesheet 2, a continuous surface 25, which is slightly elevated relative to the first surface 10, is formed by the flares and the welded connections. The continuous surface 25 is ground and polished to an even and smooth surface. The continuous surface 25 may serve as a cladding layer, as it fully covers the first surface 10 of the tube sheet 2 located directly underneath it. The remaining uncovered part of the first surface may be covered by a different material to protect it from corrosion. The device shown in figure 4 maybe applied in a heat exchanger.

In fig. 5A a different embodiment is shown from that of fig. 2. In fig. 5A a protruding end portion 28 is compressed in the direction of arrow A, to obtain a ring-shaped hart 27, which can be welded along the circumference 21 thereof to the tube sheet 2 in the direction of arrow B. The ring-shaped portion 27 can also be arranged in a recess 26, as shown in fig. 5B. The recess 26 can be machined into the tube sheet 2 by any suitable operation.

In fig. 6A the compressed end portion 27 of the tube 1 has a cone shape, and in fig. 6B the compressed end portion 27 has a trumpet shape.

Fig. 7A shows an embodiment, wherein the compressed end portion 27 exhibits both a ring-shape and a cone-shape, where the ring-shaped portion of the compressed end part 27 abuts against the first surface of the tube sheet 2, while the cone-shaped part of the compressed end portion 27 is sunk into the material of the tube sheet 2.

In fig. 7B the compressed end portion 27 is the same as in fig. 7A, but completely arranged in a recess 26 at the circumference of the bore at the first surface 10.

It is evident to the skilled person, after the disclosure of the present invention herein above, that different combinations of features and embodiments are also possible within the scope of protection for the present invention. For instance, it is possible to also use relatively thick tubes, where the wall material thereof would not be in immediate danger of being pierced or penetrated as a result of a welding operation, but compressing the material of the tube to obtain a compressed end portion of increased thickness enhances the quality of a leek-free welded connection between the tubes and the tube sheet.

## Claims

1. Method for forming a connection between a tube sheet (2) and at least one tube (1) comprising :
- providing a tube sheet (2) with a first surface (10) and a second surface (11) and a number of bores (12) extending from the first surface (10) to the second surface (11),
- providing the tube (1) of a pliable or at least deformable material with an exterior shape and dimensions, which shape and dimensions enable the tube (1) to be accommodated in a corresponding bore (12),
- placing the tube (1) in the corresponding bore (12), such that an end portion (3) of the tube (1) protrudes from the side of the first surface (10) of the tube sheet (2).
- forming an end portion (3) of the tube (1) into at least a flare (20),
- making a welded connection between the tube sheet (2) and the tube (1) at the circumference (21) of the flare (20), after placing the tube (1)
**characterised in that**
flaring the protruding end portion comprises: compressing the protruding end portion (3) axially relative to the length direction of the tube (1) and thus obtaining a compressed end portion (3) of increased thickness.

2. Method according to claim 1, further comprising:
providing a recess (26) in the tube sheet (2) at the circumference of the bore (12) at the first surface (10), the recess (26) in shape and dimensioning essentially corresponding with the compressed end portion (3) of the tube (1).

3. Method according to claim 1 or 2, wherein the flare (20) has a trumpet shape.

4. Method according to claim 1 or 2, wherein the flare (20) has a cone shape.

5. Method according to claim 3 and 4, wherein the flare (20) has a form, which is a combination of a cone shape and a trumpet shape, the trumpet shape being located closer to the circumference of the flare.

6. Method according to any one of claims 2-5, wherein the recess (26) around at least one of the bores (12) at the first surface (10) is rounded and/or has the shape of a cone.

7. Method according to any one of claims 1-6, comprising : mechanically interconnecting the tube (1) and the tube sheet (2) at the latest prior to welding the flared protruding end portion (3) of the tube (1) thus providing a preliminary positional fixation of the tube and the tube sheet (2) relative to one another to be maintained during at least one of the operations of flaring the protruding end portion of the tube (1) and welding the flare (20) to the tube sheet (2).

8. Method according to claim 7, wherein interconnecting comprises: expanding the tube (1) to fit tightly in at least a part of the corresponding bore (12), which bore (12) accommodates the tube (1).

9. Method according to claim 8, comprising: expanding the tube (1) prior to flaring thereof.

10. Method according to any one of claims 1-9, further comprising testing a welded connection by means of a pressure using non-destructive testing method, that is selected from the group comprising a soap test, a He-leak test, a water pressure test.

11. Method according to any one of claims 1-10, wherein more than one tube (1) and more than one bore (12) in the tube sheet (2) are provided, which bores (12) are provided at a distance from each other, further comprising: dimensioning the protruding end portions (3) of the tubes (1) and thus the flares (20), to approximate the circumferences (21) of the flares (20) to one another, whereby the welded connections at adjacent flares (20) overlap.

12. Method according to any one of claims 1-11, further comprising grinding the surface formed by the flare (20) and the welded connection to a smooth surface and preferably polishing the smooth surface.

13. Device comprising:
- a tubesheet (2) with a first surface (10) and a second surface (11) and a number of bore (12) extending from the first surface (10) to the second surface (11),
- at least one tube (1) of a pliable material placed in a corresponding bore (12), wherein the tube (1) has a flared end portion (3) on the side of the first surface (10), which flared end portion (3) is weld-connected at its circumference (21) to the first surface (10) of the tube sheet (2),
**characterised in that**
the flared end portion (3) is axially compressed relative to the length direction of the tube (1), whereby a compressed end portion (3) of increased thickness at least axially relative to the tube (1) is obtained.

14. Device according to claim 13, wherein a recess (26) in the tube sheet (2) is provided at the circumference of the bore (12) at the first surface (10), the recess (26) in shape and dimensioning essentially corresponding with the compressed end portion (3) of the tube (1).

15. Device according to claim 13 or 14, wherein the flare (20) has a trumpet shape.

16. Device according to claim 13 or 14, wherein the flare (20) has a cone shape.

17. Device according to claim 15 and 16, wherein the flare (20) has a form, which is a combination of a cone shape and a trumpet shape, the trumpet shape being located closer to the circumference of the flare (20).

18. Device according to any claims 14-17, wherein the recess (26) around at least one of the bores (12) at the first surface (10) is rounded and/or has the shape of a cone.

19. Device according to any one of the claims 13-18, wherein the tube (1) is expanded in the bore (12) prior to flaring thereof.

20. Device according to any one of claims 13-19, wherein more than one tube (1) and more than one bore (12) in the tube sheet (2) are provided, which bores (12) are provided at a distance from each other, wherein the protruding end portions (3) of the tube (1) and thus the flares (20) are dimensioned to approximate the circumferences of the flares (20) to one another, whereby the welded connections at adjacent flares (20) overlap.

21. Device according to any one of claims 13-20, further comprising grinding the surface formed by the flare (20) and the welded connection to a smooth surface and preferably polishing the smooth surface.

## Patentansprüche

1. Verfahren zur Ausbildung einer Verbindung zwischen einem Rohrboden (2) und mindestens einem Rohr (1) umfassend:
- Bilden eines Rohrbodens (2) mit einer ersten Fläche (10) und einer zweiten Fläche (11) sowie mehreren Bohrlöchern (12), die sich von der ersten Fläche (10) zur zweiten Fläche (11) erstrecken,
- Bilden des aus einem biegsamen oder zumindest verformbaren Material bestehenden Rohrs (1) mit einer Außenform und Abmessungen, durch dessen Form und Abmessungen das Rohr (1) in einem entsprechenden Bohrloch (12) aufgenommen werden kann,
- Anordnen des Rohrs (1) in dem entsprechenden Bohrloch (12) dergestalt, dass ein Endteil (3) des Rohrs (1) aus der ersten Fläche (10) des Rohrbodens (2) hervorsteht,
- Ausbilden eines Endteils (3) des Rohrs (1) in mindestens einer Aufweitung (20),
- Herstellen einer Schweißverbindung zwischen dem Rohrboden (2) und dem Rohr (1) am Umriss (21) der Aufweitung (20) nach Anbringen des Rohrs (1),
**dadurch gekennzeichnet,dass**
das Aufweiten des hervorspringenden Endteils umfasst: axiales Stauchen des hervorspringenden Endteils (3) relativ zur Längsrichtung des Rohrs (1), wodurch ein gestauchtes Endteil (3) mit höherer Dicke erhalten wird.

2. Verfahren gemäß Anspruch 1, weiterhin umfassend:
Bilden einer Aussparung (26) im Rohrboden (2) am Umriss des Bohrlochs (12) an der ersten Fläche (10), wobei die Aussparung (26) in Form und Abmessung im Wesentlichen dem gestauchten Endteil (3) des Rohrs (1) entspricht.

3. Verfahren gemäß Anspruch 1 oder 2, wobei die Aufweitung (20) eine Trompetenform aufweist.

4. Verfahren gemäß Anspruch1 oder 2, wobei die Aufweitung (20) eine konische Form aufweist.

5. Verfahren gemäß Anspruch 3 und 4, wobei die Aufweitung (20) eine Form aufweist, die eine Kombination aus konischer Form und Trompetenform ist, wobei sich die Trompetenform näher am Umriss der Aufweitung befindet.

6. Verfahren gemäß einem der Ansprüche 2 - 5, wobei die Aussparung (26) um zumindest eines der Bohrlöcher (12) an der ersten Fläche (10) gerundet ist und/oder eine Konusform aufweist.

7. Verfahren gemäß einem der Ansprüche 1 - 6, umfassend: Mechanisches Verbinden des Rohrs (1) und des Rohrbodens (2) spätestens vor dem Schweißen des aufgeweiteten vorspringenden Endteils (3) des Rohrs (1), wodurch eine vorläufige Lagefixierung des Rohrs und des Rohrbodens (2) relativ zueinander zumindest während einem der Arbeitsgänge, dem Aufweiten des vorspringenden Endteils des Rohrs (1) oder dem Schweißen der Aufweitung (29) an den Rohrboden (2), erhalten wird.

8. Verfahren gemäß Anspruch 7, wobei die Verbindung umfasst: Erweitern des Rohrs (1), um fest in zumindest einem Teil des entsprechenden Bohrlochs (12) zu passen, wobei das Bohrloch (12) das Rohr (1) aufnimmt.

9. Verfahren gemäß Anspruch 8, umfassend: Erweitern des Rohrs (1) vor dessen Aufweiten.

10. Verfahren gemäß einem der Ansprüche 1 - 9, weiterhin umfassend: Testen einer Schweißverbindung mittels Druck mit Hilfe eines nicht zerstörenden Testverfahrens, das aus einer Gruppe ausgewählt wird, die einen Seifentest, einen He-Lecktest und einen Test mittels Wasserdruck umfasst.

11. Verfahren gemäß einem der Ansprüche 1-10, wobei mehr als ein Rohr (1) und mehr als ein Bohrloch (12) im Rohrboden (2) ausgebildet sind, wobei die Bohrlöcher (12) voneinander beabstandet sind, weiterhin umfassend: Bemessen der vorspringenden Endteile (3) der Rohre (1) und damit der Aufweitungen (20), um die Umrisse (21) der Aufweitungen (20) anzunähern, wobei die Schweißverbindungen an den benachbarten Aufweitungen (20) überlappen.

12. Verfahren gemäß einem der Ansprüche 1-11,
weiterhin umfassend das Schleifen der durch die Aufweitung (20) und die Schweißverbindung gebildeten Fläche zu einer glatten Fläche und vorzugsweise das Polieren der glatten Fläche.

13. Vorrichtung umfassend:
- einen Rohrboden (2) mit einer ersten Fläche (10) und einer zweiten Fläche (11) sowie mehreren Bohrlöchern (12), die sich von der ersten Fläche (10) zur zweiten Fläche (11) erstrecken,
- zumindest ein Rohr (1) aus einem biegsamen Material, das in einem entsprechenden Bohrloch (12) angeordnet ist, wobei das Rohr ein aufgeweitetes Endteil (3) auf der ersten Fläche (10) aufweist, wobei das aufgeweitete Endteil (3) am Umriss (21) mit der ersten Fläche (10) des Rohrbodens (2) durch Schweißen verbunden ist,
**dadurch gekennzeichnet,dass**
das aufgeweitete Endteil (3) axial relativ zur Längsrichtung des Rohrs (1) gestaucht ist, wobei ein gestauchtes Endteil (3) von höherer Dicke zumindest axial zum Rohr (1) erhalten ist.

14. Vorrichtung gemäß Anspruch 13, wobei eine Aussparung (26) im Rohrboden (2) am Umriss des Bohrlochs (12) an der ersten Fläche ausgebildet ist, wobei die Aussparung (26) in Form und Abmessung im Wesentlichen dem gestauchten Endteil (3) des Rohrs (1) entspricht.

15. Vorrichtung gemäß Anspruch 13 oder 14, wobei die Aufweitung (20) eine Trompetenform aufweist.

16. Vorrichtung gemäß Anspruch 13 oder 14, wobei die Aufweitung (20) eine konische Form aufweist.

17. Vorrichtung gemäß Anspruch 15 und 16, wobei die Aufweitung (20) eine Form aufweist, die eine Kombination aus konischer Form und Trompetenform ist, wobei die Trompetenform näher am Umriss der Aufweitung (20) liegt.

18. Vorrichtung gemäß einem der Ansprüche 14 - 17, wobei die Aussparung (26) um zumindest einem der Bohrlöcher an der ersten Fläche (10) gerundet ist und/oder eine Konusform aufweist.

19. Vorrichtung gemäß einem der Ansprüche 13 - 18, wobei das Rohr (1) im Bohrloch (12) vor dessen Aufweitung erweitert wird.

20. Vorrichtung gemäß einem der Ansprüche 13 - 19,
wobei mehrere Rohre (1) und mehrere Bohrlöcher (12) im Rohrboden (2) ausgebildet sind, wobei die Bohrlöcher (12) voneinander beabstandet sind, wobei die vorspringenden Endteile (3) der Rohre (1) und damit die Aufweitungen (20) bemessen sind, um die Umrisse der Aufweitungen (20) einander anzunähern, wobei die Schweißverbindungen an den benachbarten Aufweitungen (20) überlappen.

21. Vorrichtung gemäß einem der Ansprüche 13 - 20,
weiterhin das Schleifen der durch die Aufweitung (20) und die Schweißverbindung gebildete Fläche zu einer glatten Fläche und vorzugsweise das Polieren der glatten Fläche umfassend.

## Revendications

1. Procédé de réalisation d'une liaison entre une platine à tubes (2) et au moins un tube (1) comprenant les étapes suivantes :
- fournir une platine à tubes (2) avec une première surface (10) et une seconde surface (11) et un certain nombre d'alésages (12) qui s'étendent depuis la première surface (10) vers la seconde surface (11),
- donner au tube (1) qui est constitué d'un matériau flexible ou au moins déformable une forme extérieure et des dimensions, lesquelles forme et dimensions permettent au tube (1) d'être logé dans un alésage (12) correspondant,
- placer le tube (1) dans l'alésage (12) correspondant, de façon à ce qu'une partie terminale (3) du tube (1) dépasse du côté de la première surface (10) de la platine à tubes (2),
- donner à une partie terminale (3) du tube (1) la forme d'au moins un évasement (20),
- réaliser une liaison soudée entre la platine à tubes (2) et le tube (1) au niveau de la circonférence (21) de l'évasement (20), après avoir placé le tube (1),
**caractérisé en ce que**
l'évasement de la partie terminale qui dépasse comprend les étapes de : comprimer la partie terminale qui dépasse (3) axialement par rapport à la longueur du tube (1) et obtenir ainsi une partie terminale (3) comprimée d'une épaisseur accrue.

2. Procédé selon la revendication 1, comprenant en outre l'étape de : produire un évidement (26) dans la platine à tubes (2) au niveau de la circonférence de l'alésage (12) sur la première surface (10), la forme et les dimensions de l'évidement (26) correspondant essentiellement avec la partie terminale (3) comprimée du tube (1).

3. Procédé selon la revendication 1 ou la revendication 2, dans lequel l'évasement (20) a une forme en trompette.

4. Procédé selon la revendication 1 ou la revendication 2, dans lequel l'évasement (20) a une forme de cône.

5. Procédé selon les revendications 3 et 4, dans lequel l'évasement (20) a une forme, qui est une combinaison d'une forme de cône et d'une forme en trompette, la forme en trompette étant située plus près de la circonférence de l'évasement.

6. Procédé selon l'une quelconque des revendications 2 à 5, dans lequel l'évidement (26) autour d'au moins un des alésages (12) sur la première surface (10) est arrondi et/ou a la forme d'un cône.

7. Procédé selon l'une quelconque des revendications 1 à 6, comprenant les étapes de : mettre mécaniquement en relation le tube (1) et la platine à tubes (2) au plus tard avant de souder la partie terminale (3) évasée du tube (1) qui dépasse, ce qui fournit une fixation en position préliminaire du tube et de la platine à tubes (2) l'un par rapport à l'autre, qui doit être maintenue pendant au moins une des opérations consistant à évaser la partie terminale du tube (1) qui dépasse et à souder l'évasement (20) à la platine à tubes (2).

8. Procédé selon la revendication 7, dans lequel la mise en relation comprend l'étape de : étendre le tube (1) de façon à ce qu'il s'insère étroitement dans au moins une partie de l'alésage (12) correspondant, lequel alésage (12) loge le tube (1).

9. Procédé selon la revendication 8, comprenant l'étape de : étendre le tube (1) avant de l'évaser.

10. Procédé selon l'une quelconque des revendications 1 à 9, comprenant en outre l'étape de tester la relation soudée au moyen d'une méthode de contrôles non destructifs utilisant la pression, choisie dans le groupe comportant un test savon, un test de recherche de fuites, un test de pression à l'eau.

11. Procédé selon l'une quelconque des revendications 1 à 10, dans lequel plus d'un tube (1) et plus d'un alésage (12) dans la platine à tubes (2) sont fournis, lesquels alésages (12) sont disposés à une certaine distance l'un de l'autre, comprenant en outre l'étape de : dimensionner les parties terminales (3) des tubes (1) qui dépassent et donc les évasements (20), afin d'obtenir des circonférences (21) d'évasement (20) proches les unes des autres, moyennant quoi les liaisons soudées au niveau des évasements (20) adjacents se chevauchent.

12. Procédé selon l'une quelconque des revendications 1 à 11, comprenant en outre l'étape de rectifier la surface formée par l'évasement (20) et la liaison soudée pour obtenir une surface lisse, et de préférence l'étape de polir la surface lisse.

13. Dispositif comprenant :
- une platine à tubes (2) avec une première surface (10) et une seconde surface (11) et un certain nombre d'alésages (12) s'étendant depuis la première surface (10) vers la seconde surface (11),
- au moins un tube (1) composé d'un matériau flexible placé dans un alésage (12) correspondant, dans lequel le tube (1) a une partie terminale (3) évasée sur le côté de la première surface (10), laquelle partie terminale (3) évasée est liée par soudure au niveau de sa circonférence (21) à la première surface (10) de la platine à tubes (2),
**caractérisé en ce que**
la partie terminale (3) évasée est comprimée axialement par rapport à la direction de longueur du tube (1), moyennant quoi une partie terminale (3) comprimée d'épaisseur accrue au moins axialement par rapport au tube (1) est obtenue.

14. Dispositif selon la revendication 13, dans lequel un évidement (26) dans la platine à tubes (2) est réalisé au niveau de la circonférence de l'alésage (12) sur la première surface (10), la forme et les dimensions de l'évidement (26) correspondant essentiellement avec la partie terminale (3) comprimée du tube (1).

15. Dispositif selon la revendication 13 ou la revendication 14, dans lequel l'évasement (20) a une forme en trompette.

16. Dispositif selon la revendication 13 ou la revendication 14, dans lequel l'évasement (20) a une forme de cône.

17. Dispositif selon les revendications 15 et 16, dans lequel l'évasement (20) a une forme, qui est une combinaison d'une forme de cône et d'une forme en trompette, la forme en trompette étant située plus près de la circonférence de l'évasement (20).

18. Dispositif selon l'une quelconque des revendications 14 à 17, dans lequel l'évidement (26) autour d'au moins un des alésages (12) sur la première surface (10) est arrondi et/ ou a la forme d'un cône.

19. Dispositif selon l'une quelconque des revendications 13 à 18, dans lequel le tube (1) est étendu dans l'alésage (12) avant l'évasement de celui-ci.

20. Dispositif selon l'une quelconque des revendications 13 à 19, dans lequel plus d'un tube (1) et plus d'un alésage (12) dans la platine à tubes (2) sont fournis, lesquels alésages (12) sont situés à une certaine distance l'un de l'autre, et dans lequel les parties terminales (3) des tubes (1) qui dépassent et donc les évasements (20) sont dimensionnés afin d'obtenir des circonférences d'évasement (20) proches l'une de l'autre, moyennant quoi les liaisons soudées au niveau des évasements (20) adjacents se chevauchent.

21. Dispositif selon l'une quelconque des revendications 13 à 20, comprenant en outre l'étape de rectifier la surface formée par l'évasement (20) et la liaison soudée pour obtenir une surface lisse, et de préférence l'étape de polir la surface lisse.
